



D represents a diffusion inhibiting group e.g. an aliphatic hydrocarbon radical with 5 to 20 carbon atoms, preferably with 14, 16 or 18 carbon atoms, and M represents a hydrogen atom, an alkali metal atom or an ammonium group.

Suitable compounds which give good results and which correspond to the above general formula are:

N-(2'-cetoxy-5'-sulfophenyl)-1-hydroxy-2-naphthoic acid amide sodium salt,  
 N-(2'-cetoxy-5'-sulfophenyl)-1-hydroxy-4-chloro-2-naphthoic acid amide sodium salt,  
 N-(2'-cetylmercapto-5'-sulfophenyl)-1-hydroxy-2-naphthoic acid amide sodium salt,  
 N-(2'-cetylmercapto-5'-sulfophenyl)-1-hydroxy-4-bromo-2-naphthoic acid amide sodium salt,  
 N-(2'-cetylmercapto-5'-sulfophenyl)-1-hydroxy-4-chloro-2-naphthoic acid amide sodium salt,  
 N-(2'-palmitoylamino-4'-sulfophenyl)-1-hydroxy-2-naphthoic acid amide sodium salt,  
 N-(2'-methyl cetylamino-5'-sulfophenyl)-1-hydroxy-4-chloro-2-naphthoic acid amide sodium salt,  
 N-(6'-cetyl sulfonylphenyl)-1-hydroxy-2-naphthoic acid amide-3'-sodium sulfonate,  
 N-(6'-cetyl sulfonylphenyl)-1-hydroxy-4-chloro-2-naphthoic acid amide-3'-sodium sulfonate,  
 N-(4'-cetyl sulfonylphenyl)-1-hydroxy-2-naphthoic acid amide-3'-sodium sulfonate.

These colour couplers for cyan can be prepared e.g. by the condensation of 1-hydroxy-2-naphthoic acid or its derivatives with the suitable aromatic amides according to the process described in the German patent specification 1,121,061.

Suitable mask-forming compounds which may be used in the process according to the invention are those the formulae of which are given in Table I.

TABLE I



The compounds with the Formulae 1 to 6 are not fast to diffusion. The mask-forming compounds which are not fast to diffusion can be applied in one of the processing baths e.g. the developing bath or the bleaching bath. Preferably they are incorporated into the photographic emulsion layer as bicarbonate thus being more or less fast to diffusion.

Mask-forming compounds corresponding to the above general formula can also comprise a diffusion fast making group such as a long aliphatic carbon chain. Examples of compounds which are fast to diffusion and which preferably are incorporated in the emulsion layer are given in Table II.



Although the above-mentioned mask-forming compounds are preferably used in combination with colour couplers for cyan, attention is drawn to the fact that these mask-forming compounds also oxidatively couple with colour couplers for magenta of the pyrazolone class with which dyes are obtained which mainly absorb in the wavelength region of 380  $\mu\text{m}$  to 430  $\mu\text{m}$ , thus masking in the blue region of the spectrum.

The mask-forming compounds used in the process according to the present invention are photographically inert and do not cause fog.

As an illustration for the manufacture of mask-forming compounds according to the present invention detailed examples of the preparation of these compounds as well as references to literature are given below.

## Preparation 1

1-(o-methoxy phenyl)-3-aminoguanidine hydroiodide is prepared as follows:

9 g. of N-(o-methoxy phenyl)-thiourea and 10 cm.<sup>3</sup> of methyl iodide are refluxed for 5 min. in 100 cm.<sup>3</sup> of dry acetone.

After distilling off the acetone, dry ether is added to the residue. A solid precipitate of N-(o-methoxy phenyl)-S-methyl isothiouronium iodide is obtained which is sucked off. Melting point: 125° (decomposition).

15.5 g. of the obtained thiouronium iodide in 100 cm.<sup>3</sup> of pyridine is treated for 4 days with 3 cm.<sup>3</sup> of hydrazine hydrate. After distilling off the pyridine, the solid residue is washed with isopropanol and recrystallized from acetonitrile. The obtained 1-(o-methoxyphenyl)-3-aminoguanidine hydroiodide melts at 176° C.

## Preparation 2

Compound 6 from Table I: 1-(N-4-acetyl sulphanilyl)-1-methyl-3-aminoguanidine is prepared as described by A. Greer in J. Am. Chem. Soc., 76 (1954), p. 1141-45.

## Preparation 3

1-n-hexadecyl-3-aminoguanidine hydroiodide is prepared as follows:

51 g. of dry ammonia thiocyanate and 70 cm.<sup>3</sup> of benzoyl chloride are refluxed for 5 min. in 450 cm.<sup>3</sup> of dry acetone (ref. R. Frank "Organic Synthesis" 23, 89).

55 The obtained solution containing benzoyl isothiocyanate and 145 g. of n-hexadecyl amine are refluxed for 15 min. in 2100 cm.<sup>3</sup> of dry acetone. After filtration 600 cm.<sup>3</sup> of water is added to the reaction mixture. The precipitated N-n-hexadecyl-N'-benzoyl thiourea is sucked off and recrystallized from ethanol. Melting point: 63° C.

60 125 g. of the obtained thiourea compound and 12.5 g. of sodium hydroxide dissolved in 1875 cm.<sup>3</sup> of ethanol are refluxed for 1 h. The reaction mixture is poured into water and the formed precipitate is sucked off and recrystallized from isopropanol.

65 After further recrystallization from acetonitrile or ethyl acetate the formed N-n-hexadecylthiourea melts at 140° C.

70 75 g. of N-n-hexadecylthiourea and 290 cm.<sup>3</sup> of methyl iodide are refluxed for 3 h. in 750 cm.<sup>3</sup> of acetone. The obtained precipitate is sucked off and washed with ether. After recrystallization from ethyl acetate N-n-hexadecyl-S-methyl isothiouronium iodide is obtained which melts at 87° C.

75 56 g. of the obtained thiouronium iodide and 6.8 cm.<sup>3</sup>

of hydrazine hydrate are refluxed for 2 h in 280 cm.<sup>3</sup> of ethanol. After cooling the formed precipitate is sucked off and recrystallized from acetonitrile. The obtained 1-n-hexadecyl-3-aminoguanidine hydroiodide melts at 103° C. (decomposition).

### *Preparation 4*

1-(p-cetyloxyphenyl)-3-aminoguanidine is prepared as follows:

A solution of benzoyl isothiocyanate is prepared from 8.5 g. of ammonium thiocyanate and 11.5 cm.<sup>3</sup> of benzoyl chloride in 50 cm.<sup>3</sup> of acetone as described in preparation 3. At the boiling temperature a solution of 16.7 g. of p-cetoxylaniline in 50 cm.<sup>3</sup> of acetone is dropwise added. After pouring out into water the obtained precipitate of N-(p-cetoxophenyl)-N'-benzoyl thiourea is sucked off and refluxed for 15 min. in a solution of 8 g. of sodium hydroxide in 70 cm.<sup>3</sup> of water. The saponified product precipitates immediately. The reaction mixture is neutralized and the p-cetoxophenyl thiourea is sucked off. After recrystallizing from benzene the product melts at 129° C.

3.92 g. of the obtained thiourea are refluxed with 10 cm.<sup>3</sup> of methyl iodide in 40 cm.<sup>3</sup> of dry acetone for 1 h. After cooling the formed N-(*p*-cetoxyphenyl)-S-methyl isothiouronium iodide is sucked off and washed with a little dry ether. Melting point: 116° C.

1.6 g. of the obtained thiouronium iodide are allowed to react at room temperature in 15 cm.<sup>3</sup> of pyridine, for 3 days with 0.5 cm.<sup>3</sup> of hydrazine hydrate. When pouring out into ice the formed 1-(*p*-cetoxy phenyl)-3-amino-guanidine precipitates. After sucking off and recrystallizing from acetonitrile the aminoguanidine melts at 90° C.

### *Preparation 5*

1-(*p*-cetyl sulphonyl phenyl)-3-aminoguanidine is prepared as follows:

A solution of benzoyl isothiocyanate is prepared from 18.8 g. of ammonium thiocyanate and 26.6 ccs. of benzoyl chloride in 200 ccs. of acetone as described in preparation 3. At boiling temperature a solution of 84.6 g. of p-cetysulphonyl aniline in 800 ccs. of acetone is added gradually. The reaction is completed by refluxing for still 1 hour. After cooling the reaction mixture and pouring it into water, the formed precipitate of N-(p-cetysulphonyl phenyl)-N'-benzoyl thiourea is sucked off. This product is shortly boiled with a solution of 45 g. of sodium hydroxide in 700 ccs. of water so as to saponify it to p-cetysulphonyl phenyl thiourea. Thereupon it is washed with water and recrystallized from ethyleneglycol monomethyllether. Yield: 90 g. Melting point: 158° C.

8.4 g. of this p-cetyl sulphonyl phenyl thiourea is refluxed for 2 hours with 20 ccs. of methyl iodide in 50 ccs. of dry acetone. After cooling, the precipitated N-(p-cetyl sulphonyl phenyl)-S-methyl isothiouronium iodide is sucked off and washed with dry ether. Yield: 9.6 g. Melting point: 130° C.

5.6 g. of the obtained iodide is refluxed for 1½ h. with 1 cm.<sup>3</sup> of hydrazine hydrate in 50 ccs. of methanol. By pouring the reaction mixture into water, 1-(*p*-cetyl sulphonyl phenyl)-3-aminoguanidine is obtained which is recrystallized from ethyl acetate. Yield: 4 g. Melting point: near 120° C. (with decomposition).

For carrying out the process according to the present invention, the colour couplers and mask compounds are preferably incorporated into a photographic silver halide emulsion prepared by means of the colloids usually employed therefor, such as for instance gelatin, polyvinyl alcohol, collodion or other natural or synthetic colloids. The silver halide emulsion is preferably coated on a transparent support consisting of glass, nitrocellulose, cellulose esters such as cellulose triacetate, polyester, polystyrene or another natural or synthetic resin, and forms part of a photographic material with one or more emulsion layers.

5 A multilayer photographic colour material is usually composed of the following layers which are coated onto a support; a red-sensitive emulsion layer having a colour coupler for cyan, a green-sensitive emulsion layer having a colour coupler for magenta and a blue-sensitive emulsion layer having a colour coupler for yellow. Usually there is a yellow filter composed in most of the cases of a gelatin layer containing dispersed colloidal silver, located between the blue-sensitive emulsion layer and the 10 emulsion layer sensitized to green. It is not only possible to incorporate the colour couplers into the light-sensitive silver halide emulsion layer itself but they can also be incorporated into an adjacent non-light-sensitive colloid layer or into a non-light-sensitive layer which is 15 separated from the light-sensitive emulsion layer by a wafer-permeable colloid layer.

The back side of the transparent support is usually coated with an antihalation layer.

On preparing the photographic multilayer colour material according to the present invention the mask-forming compound used in this invention is preferably incorporated into the red-sensitive silver halide emulsion layer containing a colour coupler for cyan of the naphthol type.

The mask-forming compounds according to the invention can also be used in combination with one of the mask-forming compounds described in the German patent specification 1,119,666 wherein is described how magenta coloured mask images, which mainly compensate the undesirable side-absorption in the green part of the spectrum of a cyan dye image, are obtained by oxidative coupling of a 4-aminopyrazolinone-3 compound corresponding to the following general formula:



wherein:

$R_1$  represents a lower alkyl group.

R<sub>2</sub> represents a lower alkyl group, an aryl group of the benzene series, or a substituted aryl group of the benzene series, and

$R_3$  represents a diffusion fast making aliphatic radical comprising a linear chain of at least 5 and at most 20 carbon atoms;

50 with colour couplers for cyan of the naphthol class. In this way a combination of mask-forming compounds can be chosen whereby the undesirable side-absorptions of the cyan dye image in the blue as well as in the green part of the spectrum are almost completely compensated.

The process for the manufacture of a masked photographic colour image according to the present invention proceeds as follows: a light-sensitive multilayer colour material as described above, comprising in the red-sensitive silver halide emulsion layer a colour coupler for cyan of the naphthol type as well as an oxidatively coupling mask-forming compound used in this invention, is exposed to a colour original. This exposed material is developed in a usual colour-developing bath whereby in the exposed areas of the light-sensitive emulsion layers the silver halide is reduced to silver by means of an aromatic primary amino developing agent the oxidation product of which in its turn couples with the colour coupler which is present in the emulsion layers. A cyan colour image which mainly absorbs the red light but also undesirably absorbs a little blue and green light is hereby obtained in the red-sensitive emulsion layer. The mask-forming compound in the red-sensitive layer remains unaffected during colour-development. The colour-developed material is then before or after fixing brought in an oxidative photographic bleaching bath wherein the metal-

lic silver dissolves and the mask-forming compound oxidatively couples with the colour coupler for cyan which is still available in the unexposed areas of the red-sensitive emulsion layer. In this way an orange to red dye mask image is formed, whereby the difference in absorption in the blue and green between the exposed and unexposed parts, which arises by the side-absorption in the blue and the green of the cyan dye image, is compensated.

It has to be noted that the oxidative coupling of the mask-forming compounds used in the present invention does not take place by the oxidative power of the exposed silver halide nor by the oxidative power of the oxidized colour developing agents.

The oxidative coupling whereby the mask image is formed proceeds with an alkaline oxidizing solution the oxidation power of which is preferably of the same strength as the oxidative power of the normally used photographic bleaching baths.

The following aromatic primary amino-compounds can be used as developers for such material: mono-, di- and triaminoaryl compounds, more especially N,N-di-alkyl-p-phenylenediamines, such as N,N-diethyl-p-phenylenediamine and N,N-diethyl-2-methyl-p-phenylene diamine, and derivatives thereof such as N,N-dialkyl-N'-sulphomethyl- or carboxymethyl-p-phenylenediamine. As useful monoamino-developers should be cited: aminophenols and aminocresols or their halogen derivatives and also the aminonaphthols.

The bleaching bath generally contains potassium bromide, borax, boric acid, magnesium sulphate and especially potassium ferricyanido. These elements are dissolved in precisely determined amounts of water so that a solution with a determined pH value above 7 is obtained.

The following examples illustrate the invention.

#### EXAMPLE 1

To 500 cm.<sup>3</sup> of a red-sensitized bromoiodide emulsion (2% of iodide) containing 1/6 mol of silver halide, are added 10 g. of the colour coupler: sodium salt of N-(2-n-hexadecyl sulphonyl-5'-sulpho)-phenyl-1-hydroxy-2-naphthoic acid amide dissolved in 7 cm.<sup>3</sup> of 2 N sodium hydroxide and 193 cm.<sup>3</sup> of distilled water. To this emulsion is further added 5 g. of the mask-forming compound 1-hexadecyl-3-aminoguanidine dissolved in 12.5 cm.<sup>3</sup> of N sodium hydroxide and 37.5 cm.<sup>3</sup> of ethylene glycol monomethyl ether. After acidifying with 32.5 cm.<sup>3</sup> of N acetic acid to pH 5.7 and after adding the usual ingredients such as hardeners and wetting agents, distilled water is added to the emulsion up to 1000 cm.<sup>3</sup>. This emulsion is coated on a suitable support and dried. After exposure through a grey-wedge with a constant 0.15 the material is developed for 9 min. at 20° C. in a colour-developing bath with the following composition:

|                                                   |     |
|---------------------------------------------------|-----|
| Sodium hexametaphosphate (anhydrous) -----        | 2   |
| N,N-diethyl-p-phenylene diamine hydrochloride --- | 3   |
| Sodium sulphite (anhydrous) -----                 | 4   |
| Sodium carbonate (anhydrous) -----                | 57  |
| Hydroxylamine hydrochloride (cryst.) -----        | 1.5 |
| Potassium bromide (cryst.) -----                  | 1   |
| Water to 1000 cm. <sup>3</sup> (pH=10.6).         |     |

This material is rinsed for 30 minutes at 18 to 20° C. and fixed for 5 minutes at 20° C. in a fixing bath of the following composition:

|                                          |     |
|------------------------------------------|-----|
| Sodium thiosulphate (anhydrous) -----    | 200 |
| Sodium bisulphite (anhydrous) -----      | 25  |
| Potassium alum., 24 aq. -----            | 20  |
| Sodium biacetate -----                   | 20  |
| Boric acid (anhydrous) -----             | 7.5 |
| Water to 1000 cm. <sup>3</sup> (pH=4.0). |     |

Next, the material is rinsed again for 10 minutes at 18 to 20° C. and treated for 5 minutes in a bleaching bath of the following composition:

|                                             |     |
|---------------------------------------------|-----|
| Potassium ferricyanide (cryst.) -----       | 100 |
| Potassium bromide (cryst.) -----            | 25  |
| Borax, 10 aq. -----                         | 20  |
| Boric acid (cryst.) -----                   | 5   |
| Water up to 1000 cm. <sup>3</sup> (pH=8.8). |     |

Then the material is rinsed again for 10 minutes at 18 to 20° C. and fixed for 5 minutes at 20° C. in a bath of the following composition:

|                                          |     |
|------------------------------------------|-----|
| Ethylene diamine tetraacetic acid -----  | 1   |
| Sodium thiosulphate (anhydrous) -----    | 130 |
| Sodium carbonate (anhydrous) -----       | 6   |
| Sodium bicarbonate (anhydrous) -----     | 14  |
| Sodium sulphite (anhydrous) -----        | 10  |
| Water to 1000 cm. <sup>3</sup> (pH=8.9). |     |

Rinsing is continued for another 10 minutes at 18 to 20° C. and finally the material is dried. In the exposed and processed strip, besides a cyan image also an orange-coloured mask image is formed (absorption maxima at 480 m $\mu$  and 530 m $\mu$ ), with a graduation opposed to that of the cyan image, and which compensates the undesired side-absorption of the cyan image in the blue and partly in the green.

#### EXAMPLE 2

To 1/2 kg. of a red-sensitized bromo-iodide emulsion (2% iodide) containing 1/6 mol of silver halide are added 9 g. of N-(6'-cetyl sulphonylphenyl)-1-hydroxy-2-naphthoic acid amide-3'-sodium sulfonate dissolved in a mixture of 175 cm.<sup>3</sup> of water and 6.3 cm.<sup>3</sup> of an aqueous solution of sodium hydroxide 2 N, 2 g. of 1,2-dimethyl-4-amino-5-nonylpyrazolinone-3 dissolved in 20 cm.<sup>3</sup> of ethanol with a little sodium hydroxide and 2.5 g. of 1-hexadecyl-3-aminoguanidine dissolved in 6.25 cm.<sup>3</sup> of N sodium hydroxide and 18.5 cm.<sup>3</sup> of ethylene glycol monomethyl ether. After acidifying with N acetic acid to pH 6 and after adding the usual ingredients such as hardeners and wetting agents, distilled water is added up to 1000 cm.<sup>3</sup>. After coating, this emulsion forms part of a multilayer photographic material consisting of the following superposed layers in the indicated sequence: an anti-halation layer, a transparent cellulose triacetate support, a subbing layer, the layer of the above-mentioned red-sensitized emulsion with colour coupler for cyan, a gelatin interlayer, a green-sensitized emulsion layer with colour coupler for magenta, a yellow filter layer, a blue-sensitive emulsion layer with colour coupler for yellow and at last a gelatin overcoat as antistress layer.

After exposure through a grey wedge with a constant 0.15 the photographic material is developed and further treated as in Example 1. In the red-sensitized silver halide emulsion layer, besides a cyan dye image, also a magenta and orange colored mask image is formed with a graduation opposed to that of the cyan image, and which compensates the undesired side-absorptions of the cyan dye image in the blue as well as in the green.

What we claim is:

1. A method of forming a colour corrected photographic colour image in a photographic element comprising at least one silver halide emulsion layer and a naphthol colour coupler, for cyan which on development by reaction with the oxidation product of an aromatic primary amino developing agent forms a primary cyan dye image, which absorbs a major proportion of light in one region of the visible spectrum, and undesirably absorbs a minor proportion of light in at least one other region of the visible spectrum, which method comprises treating said photographic element, after image-wise exposure and colour development, with an oxidizing solution in the pres-

ence of a 3-amino-guanidine compound corresponding to the following general formula:



5

wherein:

R is a member selected from the group consisting of hydrogen, an alkyl radical, an aralkyl radical, an aryl radical and a heterocyclic radical, and

R' is a member selected from the group consisting of hydrogen and an acyl radical,

said method comprising treating said photographic element, after image-wise exposure and colour development, with an oxidizing solution, whereby the colour coupler remaining undeveloped after said colour development reacts with said mask-forming compound to form a secondary dye image absorbing light in at least one such other region of the spectrum and having a gradation opposite to that of the primary dye image but transmitting substantially all of that light absorbed in major proportion by said primary dye image.

2. Method of forming a colour corrected image according to the method of claim 1, wherein the mask-forming compound is incorporated in a water-permeable colloid layer of the photographic element.

3. Method of forming a colour corrected image according to the method of claim 1, wherein the oxidizing solution is a photographic bleaching bath.

4. Method of forming a colour corrected image in a photographic element as in claim 1 wherein said element has superposed silver halide emulsion layers each sensitive to a different region of the visible spectrum, at least one of said layers containing said colour coupler of the naphthol type said layer containing said colour coupler containing also said mask-forming compound.

5. Method according to claim 4, wherein the silver halide emulsion layer of the photographic element containing said naphthol colour coupler for cyan is sensitive to red light and said coupler corresponds to the general formula:



wherein:

X is a member selected from the group consisting of oxygen, sulfur,



60

or sulfonyl,

Y is a member selected from the group consisting of hydrogen and halogen,

D is a group making the colour coupler molecule fast to diffusion, comprising an aliphatic hydrocarbon radical with 5 to 20 carbon atoms, and

M is a member selected from the group consisting of hydrogen, an alkali metal atom and an ammonium group.

6. Method according to claim 1, wherein the oxidizing solution is an alkaline photographic bleaching bath comprising potassium hexacyanoferrate (III).

7. Method according to claim 4, wherein said red sensitized silver halide emulsion layer of the photographic

70

element also contains a 4-amino-pyrazolinone-3 compound corresponding to the following general formula:



wherein:

R<sub>1</sub> is a lower alkyl group,

R<sub>2</sub> is a member selected from the group consisting of a lower alkyl group, an aryl group of the benzene series, and a substituted aryl group of the benzene series, and

R<sub>3</sub> is a radical rendering said compound fast to diffusion, comprising an aliphatic, linear, hydrocarbon radical of at least 5 and at most 20 carbon atoms.

8. Photographic multilayer colour material having superposed silver halide emulsion layers sensitive to different regions of the visible spectrum, at least one of said layers containing a naphthol colour coupler for cyan which is reactive with the oxidation product of an aromatic amino developing agent to form by colour development a primary cyan dye image which absorbs a major proportion of light in one region of the visible spectrum, and undesirably absorbs a minor proportion of light in at least one other region of the visible spectrum, and a mask-forming compound corresponding to the following general formula:

30



wherein:

R is a member selected from the group consisting of hydrogen, an alkyl radical, an aralkyl radical, an aryl radical and a heterocyclic radical, and

R' is a member selected from the group consisting of hydrogen, and an acyl radical.

9. Photographic multilayer colour material according to claim 8, wherein said silver halide emulsion layer containing a colour coupler for cyan of the naphthol type is sensitive to red light.

10. Photographic multilayer colour material having superposed silver halide emulsion layers sensitive to different regions of the visible spectrum as in claim 9, wherein the naphthol colour coupler for cyan contained in said red-sensitive emulsion layer has the formula:



50

wherein:

X is a member selected from the group consisting of oxygen, sulfur,

55



and sulfonyl,

Y is a member selected from the group consisting of hydrogen, and halogen,

D is a group making the colour coupler fast to diffusion selected from the group of aliphatic hydrocarbon radicals with 5 to 20 carbon atoms, and

M is a member selected from the group consisting of hydrogen, an alkali metal atom and an ammonium group, and a mask-forming compound of the formula:



75

wherein:

R is a member selected from the group consisting of hydrogen, an alkyl radical, an aralkyl radical, an aryl radical and a heterocyclic radical, and

R' is a member selected from the group consisting of hydrogen and an acyl group.

11. Photographic multilayer colour material as in claim 9 wherein said red-sensitive emulsion layer also contains a mask-forming compound of the formula:



wherein:

$R_1$  is a lower alkyl group,

$R_1$  is a lower alkyl group, and  
 $R_2$  is a member selected from the group consisting of a lower alkyl group and an aryl group of the benzene series, and

R<sub>3</sub> is a group making the mask-forming compound fast to diffusion and comprising an aliphatic, linear hydrocarbon chain of at least 5 and at most 20 carbon atoms.

12. Photographic multilayer colour material having superposed silver halide emulsion layers sensitive to different regions of the visible spectrum, wherein the red-sensitive emulsion layer contains the sodium salt of N-(2'-n-hexadecyl sulfonyl-5-sulfophenyl)-1-hydroxy-2-naphthoic acid amide and 1 - (p-n-hexadecyloxyphenyl)-3-aminoguanidine.

**References Cited by the Examiner**  
**UNITED STATES PATENTS**

UNITED STATES PATENTS

- |    |           |         |                        |       |
|----|-----------|---------|------------------------|-------|
| 15 | 2,704,710 | 3/1955  | Sprung -----           | 96-73 |
|    | 3,013,879 | 12/1961 | De Ramaix et al. ----- | 96-55 |
|    | 3,141,771 | 7/1964  | Bard et al. -----      | 96-55 |

NORMAN G. TORCHIN, *Primary Examiner.*

J. T. BROWN, *Examiner.*